

## UNITED STATES PATENT OFFICE

LEON LILIENFELD, OF VIENNA, AUSTRIA

## VEGETABLE TEXTILE MATERIAL AND PROCESS FOR PRODUCING SAME

No Drawing. Application filed July 23, 1924, Serial No. 727,809, and in Austria April 4, 1924.

This invention relates to a process for improving textile materials of vegetable origin.

According to the invention very valuable properties are conferred upon woven and spun material of vegetable origin by treating them in presence of alkalies with a halo-hydrin, for example a mono-halo-hydrin of a poly-alcohol. This process imparts to the materials a silky gloss of great brilliance and a pleasing finish of elastic feel.

The invention consists in treating with a halo-hydrin, for example a mono-halo-hydrin of a poly-alcohol, in presence of alkali, spun or woven material consisting of or containing a vegetable fibre, particularly cotton. The material may be treated with the halo-hydrin and with the alkali either simultaneously or in either sequence.

Among the alkalies which can be used, the most important are the caustic alkalies.

Alkali sulphides may, however, be used, although the results obtained are usually less satisfactory. The alkali sulphides when dissolved in water are largely hydrolyzed, giving a strong alkaline solution containing alkali hydroxide. Therefore the use of alkali sulphides involves the use of alkali hydroxides.

There may be treated according to the invention all vegetable fibres, such as linen, flax, hemp, ramie, jute, and especially cotton, in the form of pure vegetable (for example, pure cotton) or mixed goods, in the form of yarn in skeins or cops, or in the form of warps.

The textile goods consisting of or containing the vegetable fibre may be treated according to the invention either in the crude state or after a preliminary treatment (for instance, boiling, or heating under pressure with sodium carbonate solution or dilute alkali solution or both), either moistened or unmoistened, with or without removing the fatty constituents, either unbleached or after bleaching with an oxidizing or reducing bleaching agent, and with or without mercerizing. The material may also be previously prepared in known manner by treatment with a hydrolyzing or gelatinizing agent (for example with a strong mineral

acid such as sulphuric acid of 49-60° Baumé gravity, phosphoric acid of 55-57° Baumé gravity, hydrochloric acid of 24° Baumé gravity, or nitric acid of 43-45° Baumé gravity or more, with an ammoniacal solution of cupric oxide, or with a cold or hot solution of calcium thiocyanate or other thiocyanate). The preliminary treatment may also consist in a combination of two or more of these processes.

The conditions under which the process is carried out according to the invention may vary within wide limits, and the invention is not limited to the illustrative examples of its practical application which follow.

As example, the following methods of carrying out the invention are given.

The first method consists in treating the woven or spun material first with a solution of an alkali and then acting on it with a halo-hydrin, such as  $\alpha$ -monochlorhydrin or  $\alpha$ -dichlorhydrin or ethylene-chlorhydrin. The textile material may be treated with the alkali solution in various ways; for example by dipping or soaking it in a small or large excess of the solution; by dipping or soaking it in the solution and removing the excess of alkali solution by squeezing, centrifuging or the like; by impregnating it in an impregnating mill, jigger or the like; by padding it between smooth or engraved rollers in a padding-machine; by coating by means of closely engraved rollers in a Rouleaux machine, advantageously with the addition of a thickening agent; by spraying, or by any other known method.

As alkali solution there may be used, for example, a solution of caustic soda of 10-50 per cent strength; a solution of caustic soda of 12-40 per cent strength has been found very suitable.

The quantity of alkali solution with which the material is to be impregnated, or which is to be retained by the material, may be varied within wide limits. Thus, for instance, satisfactory results have been obtained when this quantity is from 2 to 10 times the weight of the textile material. As a rule, a quantity of from 2 to 4 times the

weight of the material will be found to be sufficient.

The temperature of the alkali solution may also be chosen from a wide range. Useful results are obtained at temperatures of from 5  $-10^{\circ}$  C. to  $+50^{\circ}$  C. according to the strength of the solution. Generally, if the solution is not too weak, the process may be conducted at room temperature.

10 In order that the alkali solution may penetrate the fibres thoroughly, and increase the lustre, the woven or spun material may be caused to pass between rollers during the treatment with the solution, or it may otherwise be subjected to a high pressure. If desired, the alkali solution may contain some alcohol. The textile material which has been treated with alkali is then treated with a halo-hydrin of a poly-alcohol, either immediately after the alkali treatment, or after standing (ripening) at room temperature for a short or long period, and either in the wet state or after it has previously been partly or completely dried. The halo-hydrin may 15 be brought into contact with the material which has been treated with the alkali solution either as such, or dissolved in a suitable solvent, or suspended in an indifferent medium. There may be used as a solvent 20 water, alcohol, a mixture of water and alcohol, or any other solvent. In order that the halo-hydrin may be uniformly distributed throughout the medium, it may be used, if desired, in admixture with a suitable binding 25 or thickening agent, such as starch, dextrin, 30 British gum, albumen or the like.

The halo-hydrin may be added in various ways to the material which has been treated with the solution of alkali. The material 40 may be impregnated or coated with the halo-hydrin, or a solution or emulsion thereof (in which case any excess may be removed, if desired, by pressing or centrifuging), or the halo-hydrin, or a solution or emulsion thereof 45 may be rolled into the material. Any other method may however be employed, such as spraying. In order that the distribution of the halo-hydrin throughout the textile material may be as uniform as possible, 50 the material may be passed through one or more pairs of rollers during the treatment, or may be subjected to pressure by other means.

For introducing the halo-hydrin there may 55 be used any suitable apparatus known in the art of finishing or printing textiles.

In practice, there are no limits to the quantity of the halo-hydrin which may be used. As a rule, it is sufficient to add not 60 more than one or at the most two molecular proportions of a halo-hydrin for each molecular proportion of caustic alkali, although the invention is not limited to this amount. In most cases it is sufficient to use a much 65 smaller quantity, for instance 0.3-0.75 molec-

ular proportions of a halo-hydrin or even less, for each molecular proportion of caustic alkali.

The material which has been treated with the halo-hydrin is then either directly washed soon after addition of the halo-hydrin or after it has been in contact with it for a short or long period (for example  $1/2$ -24 hours) at room temperature or at a higher temperature (for example  $50$ - $100^{\circ}$  C.), and, if desired, after previously having been dried, or it may advantageously be treated with a cold or warm solution of an inorganic or an organic acid, or of an acid salt, or of an ammonium or other salt, or with a tannin solution or a formaldehyde solution, or with any other precipitating agent known in the viscose or ammonia-copper-oxide-cellulose industries, or with a mixture of much precipitating agents and then washed and dried. It may be steamed before or after washing.

Any of the subsidiary operations usual in mercerization or proposed for this purpose may also be used in the present invention, for example lustring, pressure, mechanical beating, and the like.

In order to produce a high grade silky lustre, it is essential that the textile fibre should be stretched. It may be stretched throughout all the operations, that is, from the impregnation with the alkali solution at the commencement, to the washing and drying operation. The material may also be stretched only during the action of the alkali solution or of the halo-hydrin, or it may be stretched after the impregnation with the alkali solution, and may remain stretched during the action of the halo-hydrin, during the treatment with the acid, salt, or the like, and during the washing and optionally final drying. Or it may be stretched only after the action of the alkali solution and of the halo-hydrin, for the treatment with the acid or salt, for the washing operation, and if necessary for the drying operation. Or the stretching may be applied only during a part of the process, for instance, so that the material is stretched during the treatment with the alkali solution, during the treatment with an acid or salt, and during the final washing, but not stretched during the action of the mono-halo-hydrin.

The second method of carrying out the invention consists in reversing the order of the operations of the first method; that is to say, the textile material is first treated with the halo-hydrin as such, or with a solution or a suspension thereof, and is then introduced into the alkali solution or impregnated, coated, or sprinkled, or sprayed therewith.

Since the halo-hydribs have no action on the fibre in absence of alkali, the treatment with alkali solution may follow the treatment with the halo-hydrin at leisure. After the mate-

70

80

85

90

95

100

105

110

115

120

125

130

rial has been brought into contact with the alkali solution, the halo-hydrin is allowed to act for a certain time; this action may proceed at room temperature or at a higher temperature. In respect of the other conditions such as the quantitative proportions, the temperatures, the duration of the reaction, the stretching, and the finishing of the material, the conditions given in the first method of carrying out the process are equally applicable.

By an appropriate selection of the working conditions, there may be obtained by the present invention silk-like effects which are far superior to those which can be obtained by the usual methods of mercerization. In addition to the silky lustre, the woven or spun material possesses a finish which has a valuable, elastic feel. The silky lustre may be improved by one or more repetitions of the process.

The process according to the invention is also suitable for producing patterns, for which the following methods are of consequence:

1. Before the treatment with the alkali solution, a pattern is printed or stencilled on the material by means of a reserve paste which prevents either mechanically or chemically the absorption of the alkali solution. Materials suitable for the reserve are, for instance, albumen, gums, acids (such as acetic acid, citric acid, tartaric acid, or an inorganic acid), alum, aluminium sulphate, ammonium sulphate, or other salts. The material is then treated with alkali solution and a halo-hydrin according to the method described in illustration of the first method of carrying out the invention. This modification of the process permits the production of a lustrious pattern upon a dull background or vice versa.

2. The alkali solution, mixed with a suitable thickening agent (such as starch, denatured albumen, a cellulose-hydrate which is soluble in alkali, an alkyl- or oxyalkyl-cellulose derivative which is soluble in alkali solutions or in water, or a cellulose-hydroxy-paraffin-monocarboxylic acid or the like), is printed in any desired pattern on the woven material, which is then treated with a halo-hydrin as already described. The effects obtained resemble those obtained according to 1.

3. After treatment with the alkali solution and if necessary after drying, the material is printed with a reserve which prevents either mechanically or chemically, the reaction between the alkali-cellulose and the halo-hydrin. There may be used for this purpose, for example, an acid, albumen, kaolin, zinc-white, or the like. There may also be added to the reserve paste a dyestuff or pigment. After printing with the reserve, the material is treated with a halo-hydrin as in the first method of carrying out the invention, and is then treated with an acid or salt, and dried.

This method yields strongly lustrious effects on a less lustrious background, or vice versa.

4. Pattern effects may also be produced by impregnating the woven material with alkali solution according to the first method of carrying out the invention, then, if necessary after previously drying the material, printing it with a halo-hydrin dissolved or suspended in a suitable thickening medium (for example British gum, starch or dextrin) with or without the addition of a dyestuff, and then finishing the material according to the first method of carrying out the invention. Highly lustrious effects on a less lustrious background may thus be obtained.

5. A halo-hydrin in the form of a solution or suspension is printed on the woven material with the aid of a thickening agent, and the material is then subjected, with or without drying, to the action of the alkali solution. The effects are similar to those obtained in 3 and 4.

The following examples illustrates the invention the parts being by weight:—

(a) Bleached or unbleached cotton fabric or yarn is treated with caustic soda solution of 25-40 per cent strength for a period of from 5 minutes to 12 hours at room temperature, and the excess of the solution removed by wringing or centrifuging, until the material retains about 2½-3½ times its weight or any other desired proportion, of the solution. The impregnated material is then treated either immediately or after it has been allowed to stand for 3-72 hours, with  $\alpha$ -monochlorhydrin or  $\alpha$ -dichlorhydrin ( $\gamma$ -chloro-propylene-glycol) or ethylenechlorhydrin, either alone, or in the form of a solution of 10-50 per cent strength in alcohol, or in the form of a solution or a suspension of 10-50 per cent strength in a solution of British gum of 20-25 per cent strength. The yarn or fabric may be impregnated or coated on one or both sides with the halo-hydrin, or the solution or suspension thereof, or the halo-hydrin, or the solution or suspension thereof may be rolled on to or into the textile material. There is practically no limit to the quantity of  $\alpha$ -monochlorhydrin or  $\alpha$ -dichlorhydrin or ethylenechlorhydrin which may be incorporated with the yarn or fabric which has been impregnated with caustic soda solution. For reasons of economy, however, it is advisable to use a quantity equal to not more than  $\frac{1}{2}$  to 1 times the weight of the cotton goods, particularly as excellent effects may be obtained with this amount or even with a smaller amount. After the material has been in contact with  $\alpha$ -monochlorhydrin or  $\alpha$ -dichlorhydrin or ethylenechlorhydrin for a short period (e. g. 10 minutes), or for a longer period (for example 12 hours), it is washed and dried or introduced

into a dilute solution (for example of 10-20 per cent strength) of sulphuric or acetic acid, or into a solution of ammonium chloride or ammonium sulphate of 20-30 per cent strength, or into any other precipitating bath known in the viscose industry; it is allowed to remain in the bath for a short period (such as 5 minutes), or for a longer period (such as several hours), and is then washed and dried. The fixing agent may be applied to the fabric by sprinkling, spraying or the like. Or the cotton goods is washed, then treated with the fixing agent, again washed and dried. It may also be only washed and dried.

During the foregoing operations, the fabric or yarn should be stretched for at least a part of the time. If the duration of the action of the alkali solution and of the halo-hydrin is not too long, the material may be in the stretched condition throughout all the operations. It may, however, be stretched only during the action of the soda solution or after it has been impregnated therewith, and may remain stretched during the whole or a portion of the treatment with the halo-hydrin, and if necessary during the treatment with the acid or salt. The textile material may also be stretched during the washing operation, though this is advantageous only in respect of the silk-like lustre.

According to the process described in this example, there is obtained a high-grade, silk-like lustre, and a pleasing finish of elastic feel.

(b) The procedure is as in (a), with the exception that epichlorhydrin is used in place of  $\alpha$ -monochlorhydrin or  $\alpha$ -dichlorhydrin or ethylene-chlorhydrin.

(c) The procedure is as in (a) or (b) with the exception that the action of the halo-hydrin is carried out at raised temperature. For this purpose, the material which has been impregnated with caustic soda solution and brought into contact with the halo-hydrin is maintained for 10 minutes to 1 hour at a temperature of 50-100° C., for instance at 80° C.

(d) The procedure is as in (a), (b), or (c), with the exception that the caustic soda solution used is of 18-23 per cent strength, for example of 22.5 per cent strength instead of 25-40 per cent strength. The treated product has a very beautiful silky lustre.

(e) The procedure is as in (a), (b), (c), or (d), with the exception that the halo-hydrin, or solution or suspension thereof, preferably in the presence of British gum, is printed in the form of any desired pattern on the fabric which has been impregnated with the caustic soda solution and, if desired, dried before being printed.

per cent strength of  $\alpha$ -monochlorhydrin in water, to which there may be added a thickening agent, for instance British gum, as described in Example 1. The impregnated material is then introduced, if desired, after removal of the excess by squeezing or centrifuging, into a caustic soda solution of 30-40 per cent strength, allowed to remain in contact with this solution for a period of from 10 minutes to 2 hours and then finished as described in Example 1 (a). The fabric may be stretched during or after the treatment with the soda solution. A silky lustre is produced.

3 80

The procedure is as in any of Examples 1 (a) to 1 (d), with the exception that instead of aqueous caustic soda solution of 18-40 per cent strength there is used an alcoholic caustic soda solution of 18 per cent strength, prepared, for example, by mixing 600 parts of caustic soda solution of 30 per cent strength with 400 parts of alcohol of 96 per cent strength.

The silk-like effect is excellent.

4

The procedure is exactly as in any of the preceding examples, with the exception that the material is treated with a strong solution of sulphuric acid before being treated according to the invention. When sulphuric acid of 49-50° Baumé gravity is used, the treatment with the acid may occur at room temperature for a period of from several seconds to several minutes, or even longer. When a stronger acid is used, for example, of 52-54° Baumé gravity, the treatment may occupy only several seconds at room temperature, but a longer period if the acid be cooled to 0° C. or below.

The treatment with sulphuric acid may also precede mercerization of the fabric, the latter being effected for example, with caustic soda solution of 10 per cent strength at a low temperature or with a stronger caustic soda solution, for instance, one of 18-40 per cent strength at room temperature.

5 115

The procedure is just as in the preceding examples, with the exception that the fabric is previously mercerized by any known mercerizing process.

The finished products may be calendered, schreinered, or beetled, or the like, in known manner.

Examples for obtaining pattern effects by means of a reserve follow from those already given.

On treatment with a halo-hydrin of a poly-alcohol in the presence of an alkali the vegetable fibres are converted into hydroxy-alkyl derivatives of cellulose (in the case of

2

Bleached or unbleached cotton fabric or  
yarn is impregnated with a solution of 10

120

125

130

5  $\alpha$ -mono-chlorhydrin a 1-2-dihydroxy-propyl cellulose, in the case of ethylene chlorhydrin a hydroxy-ethyl cellulose). Whether that conversion of the fibres takes place only on the surface of the fibres or in their deeper parts also, depends partly upon the concentration and amount of the alkali solution, partly on the quantity of the halo-hydrin used and partly on the temperature.

10 Consequently, on treating the finished fabric with a mineral acid, for example, a hydro-halogen acid, (if concentrated in the cold, if diluted in the heat) a decomposition takes place, i. e. the poly-alcohol in question is liberated.

15 The expression "textile material" in the description and claims means, where the context permits, all vegetable fibres such as flax, linen, hemp, ramie, jute, and particularly 20 cotton and the like, in the form of fabric of the pure vegetable product (such as pure cotton fabric) or mixed fibre, or yarn in skeins, cops or warps.

25 The expression "agent which will precipitate oxyalkyl cellulose derivatives which are soluble in alkali" means acids, salts, acid salts, mixtures of acids and salts, in short all precipitating agents known in the viscose industry as well as organic acids or 30 aqueous solutions thereof, alcohols, tannic acids, and formaldehyde.

I claim:

1. A process for improving vegetable textile material which comprises acting upon 35 it with a halo-hydrin of a poly-alcohol in the presence of alkali metal hydroxide.

2. A process for improving vegetable textile material which comprises treating it with an alkali metal hydroxide solution and 40 a halo-hydrin of a poly-alcohol.

3. A process for improving vegetable textile material which comprises treating it with a halo-hydrin and a solution containing alkali metal hydroxide in two steps.

45 4. A process for improving vegetable textile material, which comprises treating it with a solution containing alkali metal hydroxide, and thereafter acting on it with a halo-hydrin of a poly-alcohol.

50 5. A process for improving vegetable textile material, which comprises treating it with an alkali metal hydroxide solution, and thereafter acting on it with a halo-hydrin of a poly-alcohol in presence of the alkali solution remaining in the material.

55 6. A process for improving vegetable textile material, which comprises treating it with an alkali metal hydroxide solution, thereafter removing at least a portion of the water by drying, and acting on it with a halo-hydrin of a poly-alcohol.

60 7. A process for improving vegetable textile material, which comprises treating it with an alkali metal hydroxide solution, and there-

after acting on it with a halo-hydrin of a poly-alcohol mixed with a thickening agent.

8. A process for improving vegetable textile material, which comprises treating it with an alkali metal hydroxide solution, and thereafter coating it on at least one side with a halo-hydrin of a poly-alcohol. 70

9. A process for improving vegetable textile material, which comprises treating it with a solution of an alkali metal hydroxide and thereafter coating it on at least one side with a halo-hydrin of a poly-alcohol mixed with a thickening agent. 75

10. A process for improving vegetable textile material, which comprises treating it with an alkali metal hydroxide solution and thereafter acting on it at certain parts with a halo-hydrin of a poly-alcohol. 80

11. A process for improving vegetable textile material, which comprises treating it with a solution of an alkali metal hydroxide and thereafter printing it with a halo-hydrin of a poly-alcohol mixed with a thickening agent. 85

12. A process for improving vegetable textile material, which comprises treating it at certain parts with an alkali metal hydroxide solution, and thereafter acting on it with a halo-hydrin of a poly-alcohol. 90

13. A process for improving vegetable textile material, which comprises treating it at a raised temperature in the presence of an alkali metal hydroxide with a halo-hydrin of a poly-alcohol. 95

14. A process for improving vegetable textile material, which comprises treating it with an alkali metal hydroxide solution, and thereafter acting on it at a raised temperature with a halo-hydrin of a poly-alcohol. 100

15. A process for improving vegetable textile material, which comprises treating it in the presence of an alkali metal hydroxide with a chlorhydrin of glycerine. 105

16. A process for improving vegetable textile material, which comprises treating it with an alkali metal hydroxide solution, and thereafter acting on it with a chlorhydrin of glycerine. 110

17. A process for improving vegetable textile material, which comprises treating it with an alkali metal hydroxide solution, and thereafter acting on it with  $\alpha$ -monochlorhydrin. 115

18. A process for improving vegetable textile material, which comprises treating it with an alkali metal hydroxide solution, and thereafter acting on it with a chlorhydrin of glycerine in the presence of the alkali lye remaining in the material. 120

19. A process for improving vegetable textile material, which comprises treating it with an alkali metal hydroxide solution, and thereafter acting on it at a raised temperature with a chlorhydrin of glycerine. 125

20. A process for improving vegetable textile material, which comprises acting on it in presence of an alkali metal hydroxide and of 130

- an alcohol with a halo-hydrin of a poly-alcohol.
21. A process for improving vegetable textile material, which comprises acting on it in presence of an alkali metal hydroxide with a halo-hydrin of a poly-alcohol, thereafter treating it with a material adapted to precipitate hydroxy alkyl derivatives of cellulose which are soluble in alkali, and then washing.
22. A process for improving vegetable textile material, which comprises treating it with an alkali metal hydroxide solution, thereafter acting on it with a halo-hydrin of a poly-alcohol, and thereafter treating it with a material adapted to precipitate hydroxy alkyl derivatives of cellulose, which are soluble in alkali, and then washing.
23. A process for improving vegetable textile material, which comprises treating it with an alkali metal hydroxide solution thereafter acting on it with a chlorhydrin of glycerine, thereafter treating it with a material adapted to precipitate hydroxy alkyl derivatives of cellulose, which are soluble in alkali, and thereafter washing.
24. A process for improving vegetable textile material, which comprises acting on it in presence of an alkali metal hydroxide with a halo-hydrin of a poly-alcohol, and stretching the material during at least a portion of the process.
25. A process for improving vegetable textile material, which comprises treating it with an alkali metal hydroxide solution, and thereafter acting on it with a halo-hydrin of a poly-alcohol, and stretching the material during at least a portion of the process.
26. A process for improving vegetable textile material, which comprises treating it with an alkali metal hydroxide solution, and thereafter acting on it with a halo-hydrin of a poly-alcohol, and stretching the material during the treatment with the alkali solution.
27. A process for improving vegetable textile material, which comprises treating it with an alkali metal hydroxide solution, and thereafter acting on it with a halo-hydrin of a poly-alcohol, and stretching the material during a portion of the treatment with the alkali solution.
28. A process for improving vegetable textile material, which comprises treating it with an alkali metal hydroxide solution, and thereafter acting on it with a chlorhydrin of glycerine, and stretching the material during at least a portion of the process.
29. A process for improving vegetable textile material, which comprises treating it with an alkali metal hydroxide solution, and thereafter acting on it with a chlorhydrin of glycerine, and stretching the material during the treatment with the alkali solution.
30. A process for improving vegetable textile material, which comprises treating it with an alkali metal hydroxide solution, and thereafter acting on it with a chlorhydrin of glycerine, and stretching the material during a portion of the treatment with the alkali solution.
31. A process for improving vegetable textile material, which comprises treating it with an alkali metal hydroxide solution, thereafter acting on it with a halo-hydrin of a poly-alcohol, thereafter treating it with a material adapted to precipitate hydroxy alkyl derivatives of cellulose, which are soluble in alkali, and thereafter washing, and stretching the material during at least a portion of the process.
32. A process for improving vegetable textile material, which comprises treating it with an alkali metal hydroxide solution, thereafter acting on it with a chlorhydrin of glycerine, then treating it with a material adapted to precipitate hydroxy alkyl derivatives of cellulose, which are soluble in alkali, and washing, and stretching the material during at least a portion of the process.
33. As new products, vegetable textile materials which have a silk-like lustre and which contain an hydroxy alkyl derivative of cellulose.
34. As new products, vegetable textile materials which have a silk-like lustre and which contain a 1-2 dihydroxy-propyl-cellulose.
35. As new products, vegetable textile materials which have a silk-like lustre and which on decomposition with a hydrogen halide yield a poly-alcohol.
36. As new products, vegetable textile materials which have a silk-like lustre and which on decomposition with a hydrogen halide yield glycerine.
37. Cellulosic textile material having generated in its fibres an hydroxy alkyl derivative of cellulose.
38. The process of improving cellulosic textile material which comprises converting it in part into a derivative of cellulose by the action of a halo-hydrin in the presence of caustic alkali.
39. The process of imparting a silky effect to vegetable textile material which comprises generating in said material from a part thereof a cellulose derivative by the action of a halo-hydrin in the presence of an alkali metal hydroxide.
40. Cellulosic textile material having generated in its fibres a derivative of cellulose which on treatment with a strong hydrogen halide decomposes into a poly alcohol.
- In testimony whereof I affix my signature.  
DR. LEON LILIENFELD.